# EUROPEAN PATENT SPECIFICATION

(11) **EP 0 327 559 B1**
(45) Date of publication and mention of the grant of the patent: **02.09.1992**
(21) Application number: 87906884.9
(22) Date of filing: 25.09.1987
(51) Int. Cl.: C10L 1/18, C10L 1/26, C10L 1/30, C07F 7/00, C10L 10/06

(54) **TITANIUM AND ZIRCONIUM COMPLEXES, AND FUEL COMPOSITIONS**
TATANIUM- UND ZIRKONIUM-KOMPLEXE UND BRENNSTOFFZUSAMMENSETZUNGEN
COMPLEXES DE TITANE ET DE ZIRCONIUM ET COMPOSITIONS POUR CARBURANTS

(30) Priority: 02.10.1986 US 914382
(43) Date of publication of application: 16.08.1989
(73) Proprietor: The Lubrizol Corporation, Wickliffe, Ohio 44092 (US)
(72) Inventor: HILL, George, Robert, Chagrin Falls, OH 44022 (US); DI BIASE, Stephen, A., Euclid, OH 44132 (US); DETAR, Marvin, Bradford, Wickliffe, OH 44092 (US)
(74) Representative: Crisp, David Norman
(86) International application number: US8702495
(87) International publication number: WO8802392

(56) References cited:
- EP-A- 0 035 649
- EP-A- 0 073 615
- EP-A- 0 092 755
- EP-A- 0 092 756
- EP-A-00 167 857
- FR-A- 1 159 705
- FR-A- 1 179 418
- FR-A- 1 194 036
- FR-A- 1 341 731
- US-A- 2 151 432
- US-A- 3 134 737
- US-A- 3 355 270
- US-A- 3 993 835
- US-A- 4 077 941
- US-A- 4 093 614
- US-A- 4 131 554
- US-A- 4 505 718
- Chemical Abstracts, volume 96, no. 10, March 1982, (Columbus, Ohio, US), W.W. Haskell et al.: "Antiknock compounds for unleaded gasolines: organic titanates"

## Description

This invention relates to a method of operating diesel engines equipped with an exhaust system particulate trap, to fuel compositions useful in operating diesel engines, and to certain titanium and zirconium complexes which are useful in the method and fuel of the invention. The fuels and titanium or zirconium compounds of the invention are useful in operating diesel engines and are effective in lowering the ignition temperature of exhaust particulates collected in the particulate traps of diesel exhaust systems.

Diesel engines have been employed as engines for over-the-road vehicles because of relatively low fuel costs and improved mileage. However, because of their operating characteristics, diesel engines discharge a larger amount of carbon black particles or very fine condensate particles or agglomerates thereof as compared to the gasoline engine. These particles or condensates are sometimes referred to as "diesel soot", and the emission of such particles or soot results in pollution and is undesirable. Moreover, diesel soot has been observed to be rich in condensed, polynuclear hydrocarbons, and some of these have been recognized as carcinogenic. Accordingly, particulate traps or filters have been designed for use with diesel engines that are capable of collecting carbon black and condensate particles.

Conventionally, the particulate traps or filters have been composed of a heat-resistant filter element which is formed of porous ceramic or metal fiber and an electric heater for heating and igniting carbon particulates collected by the filter element. The heater is required because the temperatures of the diesel exhaust gas under normal operating conditions are insufficient to burn off the accumulated soot collected in the filter or trap. Generally, temperatures of about 450-600°C are required, and the heater provides the necessary increase of the exhaust temperature in order to ignite the particles collected in the trap and to regenerate the trap. Otherwise, there is an accumulation of carbon black, and the trap is eventually plugged. The above-described heated traps do not provide a complete solution to the problem because the temperature of the exhaust gases is lower than the ignition temperature of carbon particulates while the vehicle runs under normal conditions, and the heat generated by the electric heater is withdrawn by the flowing exhaust gases when the volume of flowing exhaust gases is large. Alternatively, higher temperatures in the trap can be achieved by periodically enriching the air/fuel mixture burned in the diesel engine thereby producing a higher exhaust gas temperature.

It also has been suggested that the particle build-up in the traps can be controlled by lowering the ignition temperature of the particulates so that the particles begin burning at the lowest possible temperatures. One method of lowering the ignition temperature involves the addition of a combustion improver to the exhaust particulate, and the most practical way to effect the addition of the combustion improver to the exhaust particulate is by adding the combustion improver to the fuel. Manganese or copper compounds have been suggested as combustion improvers for fuels and fuel oils.

U.S. Patent 4,505,718 describes the treatment of lubricating oils and fuels to improve various properties thereof. When added to fuels, the combustion characteristics of the fuels are improved. The organic acids utilized to make the transition metal salts may be sulfonic acids, carboxylic acids, and phosphorus acids. The addition of transition metal salts of mixed organic carboxylic and sulfonic acids as anti-knock agents, combustion improvers and smoke suppressants is described in U.S. Patent 4,162,986. Manganese soaps and fuels are described in U.S. Patent 3,762,890, and organic magnesium compounds as fuel conditioners are described in U.S. Patent 4,202,671. Various titanium containing organic salts have been described as being useful in fuels, lubricants, etc., in, for example, U.S. Patents 4,093,614; 4,077,941; 3,355,270; and 3,493,508.

According to one aspect of the present invention there is provided a fuel composition comprising a major amount of a normally liquid fuel and a minor, property-improving amount of at least one titanium or zirconium complex effective in lowering the ignition temperature of exhaust particulates collected in the particulate traps of diesel exhaust systems, characterized by the formula:

(RO)ₓM(Ch)_{y} (I)

wherein R is hydrogen or a hydrocarbyl group containing from 1 to 30 carbon atoms; M is titanium or zirconium; x is 1 or 2; y is 2 or 3; x + y is 4; and, Ch is derived from at least one metal chelating agent.

According to another aspect of the present invention there is provided a titanium or zirconium complex characterized by the formula:

(RO)ₓM(Ch)_{y} (I)

wherein R is hydrogen or a hydrocarbyl group containing from 1 to 30 carbon atoms; M is titanium or zirconium; x is 1 or 2; y is 2 or 3; x + y is 4; and Ch is derived from a metal chelating agent selected from the group consisting of:
(A) aromatic Mannich bases, which are the reaction products of (A-1) a hydrocarbon-substituted aromatic phenol or thiol phenol, (A-2) an aldehyde or ketone, and (A-3) an amine which contains at least one primary or secondary amino group.

According to another aspect of the present invention there is provided a fuel additive concentrate comprising a normally liquid organic diluent and from 10% to 99% by weight of the complex according to the present invention.

According to yet another aspect of the present invention there is provided a method of operating a diesel engine equipped with an exhaust system particulate trap to reduce the build-up of exhaust particles collected in said trap comprising operating said diesel engine with a fuel according to the present invention.

According to a further aspect of the present invention there is provided a method of operating a diesel engine equipped with an exhaust system particulate trap to reduce the build-up of exhaust particles collected in said trap comprising operating said diesel engine with a fuel containing at least one of the titanium or zirconium complexes according to the present invention.

Various preferred features and embodiments of the present invention will now be described by way of non-limiting example.

In one embodiment, the invention relates to a method of operating a diesel engine equipped with an exhaust system particulate trap to reduce the build-up of exhaust particles collected in the trap. The method comprises operating the diesel engine with a fuel containing at least one compound according to the present invention effective to lower the ignition temperature of the exhaust particulates collected in the said trap.

The titanium and zirconium compounds according to the present invention are titanium and zirconium complexes characterized by the formula

(RO)ₓM(Ch)_{y} (I)

wherein R is hydrogen or a hydrocarbyl group containing from 1 to about 30 carbon atoms; M is titanium or zirconium; x is 1 or 2; y is 2 or 3; x + y is 4; and Ch is derived from at least one metal chelating agent. The metal chelating agents used in the preparation of the complexes (I) generally contain a hydrocarbon linkage and at least two functional groups on different carbon atoms. Generally, the functional groups are in vicinal or beta position to each other on the carbon skeleton of the hydrocarbon linkage. The hydrocarbon linkage may be aliphatic, cycloaliphatic or aromatic.

The term "metal chelating agent" is the accepted terminology for a well known class of chemical compounds which have been described in several texts including Chemistry of the Metal Chelate Compounds, by Martell and Calvin, Prentice-Hall, Inc., N.Y. (1952). Examples of functional groups which may be present in the chelating agent include hydroxy groups, carboxy groups, carbonyl groups, amino groups, or mercapto groups. Generally, the chelating agent (Ch) may be aliphatic in nature and selected from the group consisting of diols, dithiols, mercapto alcohols, diamines, amino alcohols, aminothiols, ortho-aminophenol, dicarboxylic acids, hydroxy carboxylic acids, mercapto carboxylic acids, amino carboxylic acids, diketones, ketocarboxylic acids or esters, etc. Examples of general classes of aromatic chelating agents include dihydroxy benzenes, dimercapto benzenes, mercaptohydroxy benzenes, diamino benzenes, aminohydroxy benzenes, aminomercapto benzenes, hydroxy-carboxy benzenes, aminocarboxy benzenes and mercapto-carboxy benzenes having the two functional groups in vicinal or beta position to one another on the benzene nucleus.

The titanium and zirconium complexes represented by Formula I generally are prepared by reacting one or more chelating agents with a titanium or zirconium compound represented by the formula

M(OR)₄

wherein M is titanium or zirconium and each R group is independently hydrogen or a hydrocarbyl group containing from 1 to about 30 carbon atoms. Generally, all of the R groups are hydrocarbyl groups. The number of chelate groups (Ch) which enter into the complex is dependent upon the relative amounts of the reactants, and generally, either two or three equivalents of the chelating group are reacted with two or one equivalents (respectively) of the compound of the formula M(OR)₄. The mixtures generally are heated to accelerate the reaction and to remove the alcohol (ROH) formed in the reaction.

The preferred complexes represented by Formula I are soluble in fuel, and the chelating agents accordingly are selected to impart fuel-solubility to the complex. Generally, the chelating agents will contain a carbon skeleton of from 2 to about 18 carbon atoms.

Examples of suitable metal chelating agents within the above-described groups include vicinal- and beta-diols such as ethylene glycol and 2-ethyl-1,3-hexanediol; vicinal- and beta-dithiols such as ethylene mercaptan and 1,3-propanediol; vicinal- and beta-mercapto alcohols such as beta-mercaptoethanol, 3-mercapto-1-propanol; vicinal- and beta-diamines such as ethylene diamine and propylene diamine; vicinal- and beta-amino alcohols such as ethanolamine and 3-amino-1-propanol; vicinal- and beta-aminothiols such as thioethanolamine and 3-amine-1-mercaptopropane; vicinal- and beta-dicarboxylic acids such as oxalic acid and malonic acids vicinal- and beta-hydroxy carboxylic acids such as glycolic acid and beta-hydroxy butyric acid; vicinal-and beta-mercapto carboxylic acids such as thioglycolic acid and beta-mercapto butyric acid; vicinal- and beta-amino carboxylic acids such as glycine and beta-aminobutyric acid; beta-diketones such as acetylacetone and benzoyl acetone; beta-keto carboxylic acid esters such as ethylacetoacetate; etc.

As mentioned above, the metal chelating agents also may be alicyclic chelating agents or aromatic chelating agents such as represented by the structural formula
wherein R¹ is a hydrocarbyl group containing 1 to about 100 carbon atoms, n is an integer from 0 to 4, Y is in the ortho or meta positions relative to X, and X and Y are each independently functional groups such as OH, NH₂, NHR, SH, COOR, or C(O)H wherein R is hydrogen or a hydrocarbyl group, preferably a lower aliphatic group. Specific examples of such aromatic compounds include hydrocarbyl-substituted and unsubstituted vicinal-di-hydroxy aromatic compounds such as pyrocatechol and 4-t-butyl-pyrocatechol; vicinal-dimercapto-aromatic compounds such as thiocatechol; vicinal-mercapto-hydroxyaromatic compounds such as monothio-catechol or a mercaptohydroxy benzene; vicinal-diamino-aromatic compounds such as orthophenylenediamine; vicinal-amino-hydroxyaromatic compounds such as ortho-aminophenol; vicinal-aminomercapto aromatic compounds such as orthoaminothiophenol; vicinal-hydroxycarboxy aromatic compounds such as salicyclic acid; vicinal-aminocarboxy aromatic compounds such as orthoaminobenzoic acid; vicinal-mercaptocarboxy aromatic compounds such as ortho-mercaptobenzoic acid, etc. Specific examples of alicyclic compounds include 1,2-dihydroxycyclohexane and, amino, 2-hydroxycyclohexane. The above-described alicyclic and aromatic chelating agents may have various other ring substituents including aromatic and substituted aromatic rings; hydroxy, alkoxy, and aryloxy groups, sulfhydryl, alkylthioether, arylthioether, alkylthioester, and arylthioester groups; acyl, aroyl, thioacyl and thioaroyl groups; amino, alkylamino, aryl- amino, acylamido and aroylamido groups; and nitro, halogen and sulfato groups.

In another embodiment of the present invention, the metal chelating agent (Ch) may be selected from the group consisting of:
(A) aromatic Mannich bases,
(B) amino acid compounds of the formula wherein R₁ is hydrogen or a hydrocarbyl group; R₂ is R₁ or an acyl group; R₃ and R₄ are each independently hydrogen or lower alkyl groups; and z is 0 or 1,
(C) beta diketones,
(D) phenolic compounds of the structure wherein each R is a hydrocarbyl group; and X is CH₂, S, or CH₂OCH₂, and
(E) an aromatic difunctional compound of the formula wherein R¹ is a hydrocarbyl group containing 1 to about 100 carbon atoms, n is an integer from 0 to 4, Y is in the ortho or meta-position relative to X, and X and Y are each independently OH, NH₂, NHR, COOR, SH or C(O)H groups wherein R is hydrogen or a hydrocarbyl group.

### (A): Aromatic Mannich Bases:

The Mannich reaction between active hydrogen compounds, aldehydes such as formaldehyde and amino compounds is well known. The Mannich condensation products utilized in the present invention are those which are derived from hydroxy aromatic compounds, amines or hydroxy amines, and aldehydes or ketones.

In one embodiment, the metal chelating agent (Ch) is an aromatic Mannich base which is the reaction product of (A-1) a hydrocarbon-substituted aromatic phenol or thiol phenol, (A-2) an aldehyde or ketone, and (A-3) an amine which contains at least one primary or secondary amino group.

In one embodiment, the metal chelating agent (Ch) is an aromatic Mannich base which is the reaction product of
(A-1) a compound having the formula wherein Ar is an aromatic group or a coupled aromatic group; wherein m is 1, 2 or 3; wherein n is an integer from 1 to 4; wherein R¹ independently is hydrogen or a hydrocarbyl having from 1 to about 100 carbon atoms; and wherein R° is hydrogen, amino, or carboxyl; and wherein X is O, S, or both when m is 2 or greater,
(A-2) a compound having the formula or a precursor thereof; wherein R² and R³ independently are hydrogen, a saturated hydrocarbon group having from 1 to about 18 carbon atoms; or wherein R³ is a carbonyl-containing hydrocarbon group having from 1 to about 18 carbon atoms; and
(A-3) an amine which contains at least one primary or secondary amino group.

The (A-1) hydrocarbyl-substituted hydroxyl and/or thiol-containing aromatic compound of the present invention generally has the formula (R¹)ₙ-Ar-(XH)ₘ wherein Ar is an aromatic group such as phenyl or polyaromatic group such as naphthyl, and the like. Moreover, Ar can be coupled aromatic compounds such as naphthyl, phenyl, etc., wherein the coupling agent is O, S, CH₂, a lower alkylene group having from 1 to about 6 carbon atoms, NH, and the like with R¹ and XH generally being pendant from each aromatic group. Examples of specific coupled aromatic compounds include diphenylamine, diphenylmethylene and the like. The number of "m" XH groups is usually from 1 to 3, desirably 1 or 2, with 1 being preferred. The number of "n" substituted R¹ groups is usually from 1 to 4, desirably 1 or 2 with a single substituted group being preferred. X is 0 and/or S with 0 being preferred. That is, if m is 2, X can be both 0, both S, or one 0 and one S. R¹ can be a hydrogen or a hydrocarbyl-based substituent having from 1 to about 100 carbon atoms. As used herein and throughout this specification, the term "hydrocarbyl-based substituent" or "hydrocarbyl" denotes a substituent having carbon atoms directly attached to the remainder of the molecule and having predominantly hydrocarbyl character within the context of this invention. Such substituents include the following:
(1) Hydrocarbon substituents, that is, aliphatic (for example alkyl or alkenyl), alicyclic (for example cycloalkyl or cycloalkenyl) substituents, aromatic-, aliphatic- and alicyclic-substituted aromatic nuclei and the like, as well as cyclic substituents wherein the ring is completed through another portion of the molecule (that is, any two indicated substituents may together form an alicyclic radical).
(2) Substituted hydrocarbon substituents, that is, those containing non-hydrocarbon radicals which, in the context of this invention, do not alter the predominantly hydrocarbyl character of the substituent. Those skilled in the art will be aware of suitable radicals (e.g., halo, (especially chloro and fluoro), amino, alkoxyl, mercapto, alkylmercapto, nitro, nitroso, sulfoxy, etc.)
(3) Hetero substituents, that is, substituents which, while predominantly hydrocarbon in character within the context of this invention, contain atoms other than carbon present in a chain or ring otherwise composed of carbon atoms.

As noted above, R¹ is hydrogen, or a hydrocarbyl group. The hydrocarbyl groups may contain from 1 to about 100 carbon atoms such as an alkyl, or alkyl groups may be mixtures of alkyl groups having from 1 up to an average of about 70 carbon atoms, more desirably from about 7 to about 20 carbon atoms, an alkenyl having 2 to about 30 carbon atoms, more desirably from about 8 to about 20 carbon atoms, a cycloalkyl having from 4 to about 10 carbon atoms, an aromatic group having from about 6 to about 30 carbon atoms, an aromatic-substituted alkyl or alkyl-substituted aromatic having a total of from about 7 to about 30 carbon atoms and more desirably from about 7 to about 12 carbon atoms. The hydrocarbyl-based substituent preferably is an alkyl having from 7 to about 20 carbon atoms with from about 7 to about 14 carbon atoms being highly preferred. Examples of suitable hydrocarbyl-substituted hydroxyl-containing aromatics include the various naphthols, and more preferably, the various alkyl-substituted catechols, resorcinols, and hydroquinones, the various xylenols, the varous cresols, aminophenols, and the like. Examples of various suitable (A) compounds include heptylphenol, octylphenol, nonylphenol, decylphenol, dodecylphenol, tetrapropylphenol, eicosylphenol, and the like. Dodecylphenol, tetrapropylphenol and heptylphenol are especially preferred. Examples of suitable hydrocarbyl-substituted thiol-containing aromatics include heptylthiophenol, octylthiophenol, nonylthiophenol, dodecylthiophenol, tetrapropylthiophenol, and the like. Examples of suitable thiol and hydroxyl-containing aromatics include dodecylmonothioresorcinol.

The aldehyde or ketone (A-2) used in the present invention has the formula
or a precursor thereof, wherein R² and R³ independently can be hydrogen, a hydrocarbon such as an alkyl having from 1 to about 18 carbon atoms and more preferably 1 or 2 carbon atoms. The hydrocarbon can also be a phenyl or an alkyl-substituted phenyl having from 1 to about 18 carbon atoms and more preferably from 1 to about 12 carbon atoms. Examples of suitable (A-2) compounds include the various aldehydes and ketones such as formaldehyde, acetaldehyde, propionaldehyde, butyraldehyde, valeraldehyde, benzaldehyde, and the like, as well as acetone, methyl ethyl ketone, ethyl propyl ketone, butyl methyl ketone, glyoxal, glyoxylic acid, and the like. Precursors of such compounds which react as aldehydes under reaction conditions of the present invention can also be utilized and include paraformaldehyde, formalin, trioxane and the like. Formaldehyde and its polymers, for example, paraformaldehyde are preferred. Mixtures of the various (A-2) reactants also can be utilized.

The third reactant used in preparing the Mannich base is (A-3) an amine which contains at least one primary or secondary group. Thus the amine is characterized by the presence of at least one -N-H group. The remaining valences of the above nitrogen atom preferably are satisfied by hydrogen, amino, or organic groups bonded to said nitrogen atom through direct carbon-to-nitrogen linkages. The compound may be a hydrocarbyl amine containing from zero to 10 hydroxyl and thiol groups and from 1 to 10 amine groups.

The amine (A-3) may be represented by the formula
wherein R¹ is a hydrocarbyl group, amino-substituted hydrocarbyl, hydroxy-substituted hydrocarbyl, or alkoxy-substituted hydrocarbyl group, and R² is hydrogen or R¹. Thus, the compounds from which the nitrogen-containing group may be derived include principally ammonia, aliphatic amines, aliphatic hydroxy or thioamines, aromatic amines, heterocyclic amines, or carboxylic amines. The amines may be primary or secondary amines and may also be polyamines such as alkylene amines, arylene amines, cyclic polyamines, and the hydroxy-substituted derivatives of such polyamines.

Specific amines of these types are methylamine, N-methyl-ethylamine, N-methyl-octylamine, N-cyclohexylaniline, dibutylamine, cyclohexylamine, aniline, di(p-methyl)amine, dodecylamine, octadecylamine, o-phenylenediamine, N,N'-di-n-butyl-p-phenylenediamine, morpholine, piperazine, tetrahydropyrazine, indole, hexahydro-1,3,5-triazine, 1-H-1,2,4-triazole, melamine, bis-(p-aminophenyl)methane, phenyl-methylenimine, menthanediamine, cyclohexamine, pyrrolidine, 3-amino-5,6-diphenyl-1,2,4-triazine, ethanolamine, diethanolamine, quinonediimine, 1,3-indandiimine, 2-octadecylimidazoline, 2-phenyl-4-methyl-imidazolidine, oxazolidine, and 2-heptyl-oxazolidine.

The hydroxyl-containing amines can be characterized by the formula
wherein each of the R¹ groups is independently a hydrogen atom or a hydrocarbyl, hydroxyhydrocarbyl, aminohydrocarbyl, or hydroxyaminohydrocarbyl group provided that at least one of R¹ is a hydroxyhydrocarbyl or a hydroxyaminohydrocarbyl group, R² is an alkylene group, and x is an integer from 0 to about 5.

Examples of specific hydroxyl-containing amines include ethanolamine, 2-amino-1-butanol, 2-amino-2-methyl-1-propanol, di-(3-hydroxypropyl)-amine, 3-hydroxybutyl-amine, 4-hydroxybutyl-amine, 2-amino-1-butanol, 2-amino-2-methyl-1-propanol, 2-amino-1-propanol, 3-amino-2-methyl-1-propanol, 3-amino-1-propanol, 2-amino-2-methyl-1,3-propanediol, 2-amino-2-ethyl-1,3-propanediol, diethanolamine, di-(2-hydroxypropyl)-amine, N-(hydroxypropyl)-propylamine, N-(2-hydroxyethyl)-cyclohexylamine, 3-hydroxycyclopentylamine, N-hydroxyethyl piperazine, and the like.

The amine (A-3) also may be a polyamine conforming for the most part to the formula
wherein n is an integer preferably less than about 10, A is a substantially hydrocarbon or hydrogen group, and the alkylene group is preferably a lower alkylene group having less than about 8 carbon atoms. The alkylene amines include principally methylene amines, ethylene amines, butylene amines, propylene amines, pentylene amines, hexylene amines, heptylene amines, octylene amines, other polymethylene amines, and also the cyclic and the higher homologues of such amines such as piperazines and amino-alkyl-substituted piperazines. They are exemplified specifically by: ethylene diamine, triethylene tetramine, propylene diamine, decamethylene diamine, octamethylene diamine, di(heptamethylene)triamine, tripropylene tetramine, tetraethylene pentamine, trimethylene diamine, pentaethylene hexamine, di(trimethylene)-triamine, 2-heptyl-3-(2-aminopropyl)imidazoline, 4-methyl-imidazoline, 1,3-bis(2-aminoethyl)imidazoline, pyrimidine, 1-(2-aminopropyl)piperazine. 1,4-bis(2-aminoethyl)piperazine, and 2-methyl-1-(2-aminobutyl)piperazine. Higher homologues such as are obtained by condensing two or more of the above-illustrated alkylene amines likewise are useful.

Hydroxyalkyl-substituted alkylene amines, i.e., alkylene amines having one or more hydroxyalkyl substituents on the nitrogen atoms, likewise are contemplated for use herein. The hydroxyalkyl-substituted alkylene amines are preferably those in which the alkyl group is a lower alkyl group, i.e., having less than about 6 carbon atoms. Examples of such amines include N-(2-hydroxyethyl)ethylene diamine, N,N'-bis(2-hydroxyethyl) ethylene diamine, 1-(2-hydroxyethyl)piperazine, monohydroxypropyl-substituted diethylene triamine, 1,4-bis(2-hydroxypropyl)piperazine, di-hydroxypropyl-substituted tetraethylene pentamine, N-(3-hydroxypropyl)tetramethylene diamine, and 2-heptadecyl-1(2-hydroxyethyl)imidazoline.

Higher homologues such as are obtained by condensation of the above-illustrated alkylene amines or hydroxyalkyl-substituted alkylene amines through amino groups or through hydroxy groups are likewise useful. It will be appreciated that condensation through amino groups results in a higher amine accompanied with removal of ammonia and that condensation through the hydroxy groups results in products containing ether linkages accompanied with removal of water.

The preparation of the Mannich compounds can be carried out by a variety of methods known in the art. One method involves adding the (A-1) hydroxyl containing aromatic compound, the (A-2) saturated aldehyde or ketone, and the (A-3) amine compound to a suitable vessel and heating to carry out the reaction. Reaction temperatures from about ambient to about the decomposition temperature of any component or the Mannich product can be utilized. During reaction, water is drawn off as by sparging. Desirably, the reaction is carried out in solvent such as an aromatic type oil. The amount of the various reactants utilized is desirably on a mole to mole basis of (A-1) and (A-2) for each (A-3) secondary amino group or on a two-mole basis of (A-1) and (A-2) for each (A-3) primary amino group, although larger or smaller amounts can also be utilized.

In another method of preparing Mannich products, the hydroxyl containing aromatic compound (A-1) and the amine compound (A-3) are added to a reaction vessel. The aldehyde or ketone (A-2) is generally rapidly added and the exothermic reaction generated is supplemented by mild heat such that the reaction temperature is from about 60°C to about 90°C. Desirably the addition temperature is less than the boiling point of water, otherwise, the water will bubble off and cause processing problems. After the reaction is essentially complete, the water by-product is removed in any conventional manner as by evaporation thereof which can be achieved by applying a vacuum, applying a sparge, heating or the like. A nitrogen sparge is often utilized at a temperature of from about 100°C to about 130°C. Naturally, higher or lower temperatures can be utilized.

The reaction is generally carried out in a solvent. Any conventional solvent can be utilized such as toluene, xylene or propanol. Oftentimes various oils are utilized such as an aromatic type oil, 100 neutral oil, etc.

Some examples of the amounts of the various (A-1), (A-2) and (A-3) components are set forth above. However, other amounts and ratios can be utilized. For example, for each primary amino group of (A-3) from about 0.5 to about 6 moles of (A-1) and (A-2) can be utilized and more desirably from about 1.8 to about 2.2 moles of (A-1) and (A-2). For each secondary amino group of (A-3), from about 0.2 to about 2 moles of (A-1) and (A-2) can be utilized and more desirably from about 0.9 to about 1.1 moles of (A-1) and (A-2).

### (B): Amino Acid Compounds

The metal chelating agent (Ch) also may be at least one amino acid compound of the formula
wherein R₁ is hydrogen or a hydrocarbyl group; R₂ is R₁ or an acyl group; R₃ and R₄ are each independently hydrogen or lower alkyl groups; and z is 0 or 1. The hydrocarbyl groups R₁ and R₂ may be any one of the hydrocarbyl groups as broadly defined above. In particular, R₁ and R₂ are alkyl, cycloalkyl, phenyl, alkyl-substituted phenyl, benzyl or alkyl-substituted benzyl groups.

In one preferred embodiment, R₁ and R₂ of Formula VI are each independently alkyl groups containing from 1 to about 18 carbon atoms, cyclohexyl, phenyl, phenyl groups containing alkyl substituents containing from 1 to about 12 carbon atoms at the 4-position of the phenyl ring, benzyl or benzyl having an alkyl group of from 1 to about 12 carbon atoms at the 4-position of the phenyl ring. Generally, R₁ in Formula VI is a lower alkyl such as a methyl group, and R₂ is an alkyl group having from about 4 to about 18 carbon atoms.

In another embodiment, R₁ is as defined above and R₂ is an acyl group. Although a variety of acyl groups may be utilized as R₂, the acyl group generally can be represented by the formula

R₂'C(O)-

wherein R₂' is an aliphatic group containing up to about 30 carbon atoms. More generally, R₂' contains from about 12 to about 24 carbon atoms. Such acyl-substituted amino carboxylic acids are obtained by reaction of an amino carboxylic acid with a carboxylic acid or carboxylic halide. For example, a fatty acid can be reacted with an amino carboxylic acid to form the desired acyl-substituted amino carboxylic acid. Acids such as dodecanoic acid, oleic acid, stearic acid, linoleic acid, etc., may be reacted with amino carboxylic acids such as represented by Formula VI wherein R₂ is hydrogen.

The groups R₃ and R₄ in Formula VI are each independently hydrogen or lower alkyl groups. Generally, R₃ and R₄ will be independently hydrogen or methyl groups, and most often, R₃ and R₄ are hydrogen.

In Formula VI, z may be 0 or 1. When z is 0, the amino acid compound is glycine, alpha-alanine and derivatives of glycine and alpha-alanine. When z is 1, the amino carboxylic acid (VI) is beta-alanine or derivatives of beta-alanine.

The amino acid compounds of Formula VI which are useful as metal chelating agents in the present invention can be prepared by methods described in the prior art, and some of these amino acids are available commercially. For example, glycine, alpha-alanine, beta-alanine, valine, arginine, and 2-methyl-alanine. The preparation of amino acid compounds represented by Formula VI where z is 1 is described in, for example, U.S. Patent 4,077,941. For example, the amino acids can be prepared by reacting an amine of the formula

R₁R₂NH

wherein R₁ and R₂ are as previously defined, with a compound of the formula

R₃CH=C(R₄)-CO₂R

₅

wherein R₃ and R₄ are as defined previously with respect to Formula VI, and R₅ is a lower alkyl, preferably methyl or ethyl, followed by hydrolysis of the ester with a strong base and acidification. Among the amines which can be reacted with the unsaturated ester are the following: dicyclohexylamine, benzylmethylamine, aniline, diphenylamine, methylethylamine, cyclohexylamine, n-pentylamine, diisobutylamine, diisopropylamine, dimethylamine, dodecylamine, octadecylamine, N-n-octylamine, aminopentane, sec-butylamine, propylamine, etc.

Amino acid compounds of Formula VI wherein R₂ is methyl or an acyl group can be prepared by reacting a primary amine of the formula

R₁NH₂

wherein R₁ is as defined previously with a compound of the formula

R₃CH=C(R₄)-CO₂R₅

wherein R₃, R₄ and R₅ are as defined above. Subsequently, this intermediate is converted to the methyl derivative by N-methylation and hydrolysis of the ester followed by acidification. The corresponding acyl derivative is formed by reacting the intermediate with an acid or acid halide such as stearic acid, oleic acid, etc. Specific amino acids of the type represented by Formula VI are illustrated in the following Table I.

### (C): Beta-Diketones

The metal chelating agent (Ch) also may be at least one beta-diketone. Generally, the beta-diketone is characterized by the formula

R-C(O)-CH₂-C(O)-R₁ (VII)

wherein R and R₁ are each independently hydrocarbyl groups. The hydrocarbyl groups may be aliphatic or aromatic hydrocarbyl groups as defined above. Among the aliphatic hydrocarbyl groups, the lower hydrocarbyl groups containing up to about 7 carbon atoms are preferred. Specific examples of R₁ and R₂ groups include methyl, ethyl, phenyl, benzyl, etc., and specific examples of beta-diketones include acetyl acetone and benzoyl acetone.

### (D): Phenolic Compounds

The metal chelating agent (Ch) also may be at least one phenolic compound of the formula
wherein each R is a hydrocarbyl group; and X is CH₂, S, or CH₂OCH₂. In one embodiment, each R is independently an aliphatic group which generally contains from about 4 to about 20 carbon atoms.

Examples of typical R groups include butyl, hexyl heptyl, 2-ethyl-hexyl, octyl, nonyl decyl, dodecyl, etc.

The phenolic compounds represented by Formula VIII can be prepared by reacting the appropriate substituted phenol with formaldehyde or a sulfur compound such as sulfur dichloride. When one mole of formaldehyde is reacted with two moles of the substituted phenol, the bridging group X is CH₂. When a molar ratio of formaldehyde to substituted phenol is 1:1, bis-phenolic compounds bridged by the group CH₂OCH₂ can be formed as a result of the reaction. When two moles of a substituted-phenol are reacted with one mole of sulfur dichloride, a bis-phenolic compound is formed which is bridged by a sulfur atom.

### (E): Aromatic Difunctional Compounds

The metal chelating agent (Ch) may be an aromatic difunctional compound of the formula
wherein R¹ is a hydrocarbyl group containing 1 to about 100 carbon atoms, n is an integer from 0 to 4, Y is in the ortho or meta position relative to X, and X and Y are each independently OH, NH₂, NR₂, COOR, SH, or C(O)H wherein R is hydrogen or a hydrocarbyl group. Specific examples of useful aromatic difunctional compounds represented by Formula IX have been given above.

In one preferred embodiment, the metal chelating agent (Ch) is an amino phenol. Preferably, the amino phenol is an ortho-amino phenol which may contain other substituent groups such as hydrocarbyl groups.

The following examples illustrate the preparation of several exemplary metal chelating agents which are useful in preparing the titanium or zirconium complexes of the present invention. Unless otherwise indicated in the following examples and elsewhere in the specification and claims, all parts and percentages are by weight, and all temperatures are in degrees centigrade.

### Example A

A mixture of 157 parts of dodecylphenol and 296 parts of mineral oil is prepared, and to this mixture there is added with stirring, 20.6 parts of a commercial polyamine mixture by responding to diethylenetriamine over a period of 30 minutes. To this mixture at about 60°C, there is added 20.6 parts of formalin solution (37% paraformaldehyde) dropwise over a period of one hour while maintaining the reaction temperature below about 96°C. The mole ratio of phenol to formaldehyde to amine is 3:3:1. After complete addition of the formalin solution, the reaction mixture is maintained at a temperature of about 96-99°C for 3.5 hours. The water formed in the reaction is removed by distillation under vacuum and thereafter cooled to room temperature. The product that is obtained is a red oil.

### Example B

Dodecylphenol (1000 parts) is charged to a reaction vessel and the temperature is adjusted to 38-55°C whereupon 290 parts of sulfur dichloride is added at a rate to maintain the temperature of the reaction mixture below about 66°C. The mixture is blown with nitrogen while heating to 143-149°C, and the mixture is maintained at this temperature until the direct acid number is less than 1.5 acid. The mixture is cooled to about 95-100°C while adding about 788 parts of diluent oil. The reaction mixture is filtered, and the filtrate is the desired sulfur-coupled phenol.

### Example C

A mixture of 526 parts (2.01 mole) of dodecylphenol, 44.1 parts (1.34 moles) of paraformaldehyde flakes, 60 parts of toluene, 90 parts of isopropyl alcohol and 3 parts of caustic soda and 12 parts of water is prepared with stirring. The mixture is heated to a temperature of about 115°C over a period of about 20 minutes to remove solvent. The mixture then is maintained at 145°C while sparging with nitrogen until no additional solvent can be removed from the mixture. The residue is the desired methylene-coupled phenolic product.

### Example D

A reaction flask is charged with 3240 parts of dodecyl phenol, 2772 parts of hydro-refined naphthenyl oil and 380 parts of ethanolamine. The mixture is stirred and heated to 72°C, and 372 parts paraformaldehyde are rapidly charged thereto. The reaction temperature is increased to a maximum of 147°C over a 3-hour period while water is removed by sparging with nitrogen. A total of 218 parts of water is collected versus a theoretical amount of 230 parts. The mixture is cooled and the product is removed. As previously described the complexes of the present invention may be prepared by the reaction of one or more titanium or zirconium compounds represented by the formula

M(OR)

₄

wherein M and R are as described above, with one or more of the metal chelating agents (Ch) described above. The metal chelating compound (Ch) displaces one or more of the R groups depending upon the number of equivalents of metal chelating agent utilized per equivalent of titanium or zirconium compound. For example, if one equivalent of the metal compound M(OR)₄ is reacted with two equivalents of the metal chelating agent, then x and y in Formula I are each 2. Similarly, if one equivalent of the metal compound M(OR)₄ is reacted with three equivalents of the metal chelating agent, then x is 1 and y is 3 in Formula I.

The reaction between the metal compound M(OR)₄ and the metal chelating agent is affected by mixing the reactants. In many instances, the reaction is exothermic and external heating of the mixture is unnecessary. The alcohol (ROH) formed in the reaction may be left in the reaction product or removed by distillation. Alternatively, the reaction mixture can be heated to an elevated temperature to increase the rate of reaction and/or to remove the alcohol found. Generally, the reaction mixture is heated at an elevated temperature (optionally under reduced pressure) until substantially no additional alcohol can be recovered by distillation. The reaction mixture may be purged with nitrogen or other inert gas in order to facilitate the removal of the alcohol.

The following examples illustrate the preparation of the titanium complexes of Formula I.

### Example 1

To the reaction product obtained in Example A, there is added 56 parts of tetra-n-butyl titanate. This mixture is heated to 110°C at 25-30 mm. Hg. and thereafter at 150°C at 16 mm. Hg. while removing n-butanol. The residue is cooled to 60° and filtered through a filter aid. The filtrate is the desired product.

### Example 2

A mixture is prepared containing 107 parts of tetra-i-propyl titanate and 520.2 parts of a 50% xylene solution of the Mannich base prepared as in Example A except that the dodecylphenol is replaced by an equivalent amount of heptylphenol and the reaction is conducted in xylene. Upon addition of the titanium compound, the mixture turns red, and an exotherm to about 42°C in five minutes is observed. The mixture is stirred for 1.3 hours at a temperature of 35-40°C.

### Example 3

A mixture of 100 parts of isopropyl alcohol, 47.4 parts of a commercial alcohol mixture containing an average of about 9 to about 11 carbon atoms (Neodol 91, Shell Chemical), and 85.2 parts of tetraisopropyl titanate is prepared, and 30 parts of 2,4-pentanedione is added with stirring. An exothermic reaction occurs, and after a period of about several minutes, the solvent is removed by stripping. The residue, a yellow oil, is the desired titanium complex.

### Example 4

A mixture of 163 parts of tetraisopropyl titanate and 406 parts of Sarkosyl O (N-oleoyl sarkosine available from Ciba Geigy) is prepared, purged with nitrogen, and heated with stirring under vacuum to a temperature of about 55°C (about 80 mm. Hg.). The mixture then is heated to about 100°C at 70-90 mm. Hg. over a period of about 1.6 hours until no further distillate is obtained. The mixture is vacuum stripped at 100°C at about 10-20 mm. Hg. The residue is filtered at about 100°C through a filter aid. The filtrate is the desired titanium complex.

### Example 5

Into a reaction vessel there is added 604 parts of the product of Example B, and the product is stirred and heated to about 160°C in a nitrogen atmosphere. After cooling to about 60°C, 101 parts of tetraisopropyl titanate is added over a period of 5 minutes. The mixture is heated to 145°C for one hour, and 80 parts of a colorless liquid is removed by distillation. A residue is the desired titanium complex.

### Example 6

To the methylene-coupled phenolic product prepared in Example C, there is added 138 parts of a diluent oil followed by the addition of 152 parts of tetraisopropyl titanate dropwise over a period of about 6 minutes. The temperature of the reaction mixture is maintained at about 150°C for about one hour while removing about 128 parts of isopropanol. The residue is the desired titanium complex containing 20% diluent oil.

### Example 7

A mixture of 363 parts of butyl diethanolamine and 388 parts of a diluent oil is prepared and heated to about 100°C at 120 mm. Hg. whereupon 100 parts of tetraisopropyl titanate and 225 parts of tetra-n-butyl titanate are added in three portions with stirring. After reducing the pressure to 20-25 mm. Hg. at 65°C, the mixture is stirred for 1.2 hours as butyl and isopropyl alcohols are removed by distillation. The residue is filtered, and the light red-orange filtrate is the desired titanium complex containing 10.6% titanium (theory, 10.2).

The above-described titanium and zirconium compounds, and in particular, the titanium and zirconium complexes described above are particularly useful in fuel compositions which comprise a major proportion of a normally liquid fuel, usually a hydrocarbonaceous petroleum distillate fuel such as diesel fuels, distillate fuels, heating oils, residual fuels, transfer fuels, and motor gasoline as defined by ASTM Specification D-439. Diesel fuels may be defined broadly as fuels having a suitable boiling range and viscosity for use as a fuel in a diesel-type engine. Fuels containing alcohols and esters also are included within the definition of a diesel fuel. The boiling range of a diesel fuel can vary from about an ASTM boiling range of about 120°C to about 425°C, more desirably from about 140°C to about 400°C, and most often between about 200°C to about 370°C. Generally, diesel fuels are within grades 1D, 2D and 4D, and usually, the diesel fuels have viscosities of from about 1.3 to about 24.0 centistokes at 40°C.

The diesel fuel compositions which are treated in accordance with the present invention will contain an amount of the titanium and zirconium compounds described above which is effective in lowering the ignition temperature of exhaust particulates formed on burning of the diesel fuel. Thus, the fuel compositions generally will contain from 1 to about 5000 parts of titanium or zirconium per million parts of fuel, and most often, the diesel fuels will contain from about 1 to about 500 parts of titanium or zirconium per million parts of fuel.

In applications where the fuel contains some water or where the fuel may come in contact with water, it is desirable and preferable that the titanium and zirconium compounds be complexes that are hydrolytically stable. Any of the metal chelating agents described above can be included in the complexes of the present invention provided that the complex is hydrolytically stable. Preferably the Ch group is one or more of the chelate groups identified as A, B, C, D or E above.

The fuel compositions can contain, in addition to the compositions of this invention, other additives which are well known to those of skill in the art. These include antiknock agents such as tetraalkyl lead compounds, lead scavengers such as haloalkanes (e.g., ethylene dichloride and ethylene dibromide), deposit preventers or modifiers such as triaryl phosphates, dyes, cetane improvers, antioxidants such as 2,6-ditertiary-butyl-4-methyl-phenol, rust inhibitors such as alkylated succinic acids and anhydrides, bacteriostatic agents, gum inhibitors, metal deactivators, demulsifiers, upper cylinder lubricants and anti-icing agents.

In certain preferred fuel compositions the compositions of this invention are combined with an ashless dispersant in gasoline. Suitable ashless dispersants include esters of mono- or polyols and high molecular weight mono- or polycarboxylic acid acylating agents containing at least 30 carbon atoms in the acyl moiety. Such esters are well known to those skilled in the art. See, for example, French Patent 1,396,645; British Patents 981,850; 1,055,337 and 1,306,529; and U.S. Patents 3,255,108; 3,311,558; 3,331,776; 3,346,354; 3,522,179; 3,579,450; 3,542,680; 3,381,022; 3,639,242; 3,697,428; and 3,708,522. These patents are expressly incorporated herein by reference for their disclosure of suitable esters and methods for their preparation. Generally, the weight ratio of the composition of this invention to the aforesaid ashless dispersant is between about 0.1:1 and about 10:1, preferably between about 1:1 and about 10:1.

The titanium and zirconium compositions of this invention can be added directly to the fuel, or they can be diluted with a substantially inert, normally liquid organic diluent such as naphtha, benzene, toluene, xylene or a normally liquid fuel as described above, to form an additive concentrate. These concentrates generally contain from about 20% to about 90% by weight of the composition of this invention and may contain, in addition one or more other conventional additives known in the art or described hereinabove.

The following examples illustrate the fuel compositions of the invention and fuel compositions useful in this invention.

| Fuel A | |
|---|---|
| Titanium Complex of Ex. 1 | 2100 ppm |
| No. 2 Fuel Oil | remainder |

| Fuel B | |
|---|---|
| Titanium Complex of Ex. 2 | 4400 ppm |

| Fuel C | |
|---|---|
| Titanium acetonylacetonate | 100 ppm (Ti) |
| No. 1 Fuel Oil | remainder |

| Fuel D | |
|---|---|
| Titanium Complex of Ex. 4 | 125 ppm (Ti) |
| No. 2 Fuel Oil | remainder |

While the invention has been explained in relation to its preferred embodiments, it is to be understood that various modifications thereof will become apparent to those skilled in the art upon reading the specification. Therefore, it is to be understood that the invention disclosed herein is intended to cover such modifications as fall within the scope of the appended claims.

## Claims

1. A fuel composition comprising a major amount of a normally liquid diesel fuel and a minor, property-improving amount of at least one titanium or zirconium complex effective in lowering the ignition temperature of exhaust particulates collected in the particulate traps of diesel exhaust systems, characterized by the formula:
(RO)ₓM(Ch)_{y} (I)
wherein R is hydrogen or a hydrocarbyl group containing from 1 to 30 carbon atoms; M is titanium or zirconium; x is 1 or 2; y is 2 or 3; x + y is 4; and, Ch is derived from at least one metal chelating agent.

2. The fuel composition of claim 1, wherein the chelating agent (Ch) is a diol, a dithiol, a mercapto alcohol, a diamine, an amino alcohol, an amino thiol, an ortho-aminophenol, a dicarboxylic acid, a hydroxy carboxylic acid, a mercapto carboxylic acid, an amino carboxylic acid, a diketone, a ketocarboxylic acid, or ester, or mixtures thereof;
wherein the complex is a titanium complex; and,
wherein R in formula I is an aliphatic group containing from 1 to 30 carbon atoms.

3. The fuel composition of claim 1, wherein the metal chelating agent (Ch) is selected from:
(A) aromatic Mannich bases which is the reaction product of (A-1) a hydrocarbon-substituted aromatic phenol or thiol phenol, (A-2) an aldehyde or ketone, and (A-3) an amine which contains at least one primary or secondary amino group.
(B) amino acid compounds of the formula wherein R₁ is hydrogen or a hydrocarbyl group; R₂ is R₁ or an acyl group; R₃ and R₄ are each independently hydrogen or lower alkyl groups; and z is 0 or 1,
(C) beta diketones characterized by the formula;
R-C(O)-CH₂-C(O)-R₁ (VII)
wherein R and R₁ are each independently hydrocarbyl groups;
(D) phenolic compounds of the structure wherein each R is a hydrocarbyl group; and X is CH₂, S, or CH₂OCH₂, and
(E) aromatic difunctional compound of the formula: wherein R¹ is a hydrocarbyl group containing 1 to 100 carbon atoms, n is an integer from 0 to 4; y is in the ortho or meta-position relative to X; and X and Y are each independently OH, NR₂, NHR, COOR, SH or C(O)H groups wherein R is hydrogen or a hydrocarbyl group.

4. The fuel composition of claim 3,
wherein the aromatic phenol or thiophenol compound (A-1) is represented by the formula: wherein Ar is an aromatic group or a coupled aromatic group; m is 1, 2 or 3, n is an integer from 1 to 4; R¹, independently, is hydrogen or a hydrocarbyl group having from 1 to 100 carbon atoms; R° is hydrogen, amino, or carboxyl, and x is 0, S, or both when m is 2 or greater;
wherein the aldehyde or ketone (A-2) is characterized by the formula: wherein R² and R³, independently, are hydrogen, a hydrocarbon group having from 1 to 18 carbon atoms, or R³ is a carbonyl containing hydrocarbon group having from 1 to 18 carbon atoms;
wherein said (A-3) compound is a hydrocarbyl amine containing from zero to 10 hydroxyl and thiol groups and from 1 to 10 amine groups;
wherein for the amino acid (VI) R¹ is an alkyl, cycloalkyl, phenyl, alkyl-substituted phenyl, benzyl or alkyl-substituted benzyl group;
R₃ and R₄ are hydrogen; z is O; and
R₂ is an acyl group represented by the formula:
R₂'C(O)-
wherein R₂' is an aliphatic group containing up to 30 carbon atoms; and
wherein for the phenolic compound (VIII) X is CH₂,
and each R is a hydrocarbyl group containing from 4 to 20 carbon atoms.

5. The fuel composition of claim 4,
wherein R¹ of said (A-1) compound is hydrogen, an alkyl group having from 1 to an average of 70 carbon atoms, an alkenyl group having from 2 to 30 carbon atoms, a cycloalkyl group having from 4 to 10 carbon atoms, an aromatic having from 6 to 30 carbon atoms, an aromatic-substituted alkyl or an alkyl-substituted aromatic group having from 7 to 30 carbon atoms, and said coupling agent of said coupled Ar group is O,S, NH or a lower alkylene group;
wherein the amine (A-3) is at least one aliphatic or aromatic monoamine or polyamine containing at least one primary and/or secondary amino group, polyalkylene polyamine, or heterocyclic amine or polyamine.

6. The fuel composition of claim 3, wherein (A-3) is a hydroxylhydrocarbyl amine having the formula: wherein each of R¹ is independently a hydrogen atom or a hydrocarbyl, hydroxyhydrocarbyl, aminohydrocarbyl, or hydroxyaminohydrocarbyl group, provided that at least one of R¹ is a hydroxyhydrocarbyl or hydroxyaminohydrocarbyl group; R² is an alkylene group, and x is an integer from 0 to 5.

7. A titanium or zirconium complex characterized by the formula:
(RO)ₓM(Ch)_{y} (I)
wherein R is hydrogen or a hydrocarbyl group containing from 1 to 30 carbon atoms, M is titanium or zirconium; x is 1 or 2; y is 2 or 3; x + y is 4; and Ch is derived from a metal chelating agent selected from:
(A) aromatic Mannich bases, which are the reaction products of (A-1) a hydrocarbon-substituted aromatic phenol or thiol phenol, (A-2) an aldehyde or ketone, and (A-3) an amine which contains at least one primary or secondary amino group.

8. The complex of claim 7,
wherein (A-1) is represented by the formula: wherein Ar is an aromatic group or a coupled aromatic group; m is 1, 2 or 3, n is an integer from 1 to 4; R¹, independently, is hydrogen or a hydrocarbyl group having from 1 to 100 carbon atoms; R° is hydrogen, amino, or carboxyl, and X in O,S, or both when m is 2 or greater;
wherein (A-2) is characterized by the formula: or a precursor thereof wherein R² and R³, independently, are hydrogen, a hydrocarbyl group having from 1 to 18 carbon atoms, or R³ is a carbonyl containing hydrocarbon group having from 1 to 18 carbon atoms;
wherein (A-3) is characterized by the formula: wherein R¹ is a hydrocarbyl, amino-substituted hydrocarbyl, hydroxy-substituted hydrocarbyl, or alkoxy-substituted hydrocarbyl group, and R² is hydrogen or R¹.

9. A fuel additive concentrate comprising a normally liquid organic diluent and from 10% to 99% by weight of the complex as claimed in any one of claims 7 and 8.

10. A method of operating a diesel engine equipped with an exhaust system particulate trap to reduce the build-up of exhaust particles collected in said trap comprising operating said diesel engine with a fuel as claimed in any one of claims 1-6.

11. A method of operating a diesel engine equipped with an exhaust system particulate trap to reduce the build-up of exhaust particles collected in said trap comprising operating said diesel engine with a fuel containing at least one of the titanium or zirconium complexes in any one of claims 7-8.

## Patentansprüche

1. Kraftstoffzusammensetzung, umfassend eine Hauptmenge eines normalerweise flüssigen Dieselkraftstoffs und eine geringere, eigenschaftverbessernde Menge mindestens eines bei der Senkung der Zündtemperatur von Abgaspartikeln, die sich in den Partikelfängern von Dieselmotorabgassystemen anreichern, wirksamen Titan- oder Zirkoniumkomplexes, der durch die Formel:
(RO)ₓM(Ch)_{y} (I)
gekennzeichnet ist, in der R ein Wasserstoffatom oder einen Kohlenwasserstoffrest mit 1 bis 30 Kohlenstoffatomen bedeutet; M ein Titan- oder Zirkoniumatom bedeutet; x 1 oder 2 ist; y 2 oder 3 ist; x + y 4 ist; und Ch sich von mindestens einem metallchelatisierenden Mittel ableitet.

2. Kraftstoffzusammensetzung nach Anspruch 1, wobei das chelatisierende Mittel (Ch) ein Diol, Dithiol, Mercaptoalkohol, Diamin, Aminoalkohol, Aminothiol, Orthoaminophenol, eine Dicarbonsäure, Hydroxycarbonsäure, Mercaptocarbonsäure, Aminocarbonsäure, ein Diketon, eine Ketocarbonsäure oder ein Ester oder ein Gemisch davon, ist; wobei der Komplex ein Titankomplex ist; und, wobei R in Formel I einen aliphatischen Rest mit 1 bis 30 Kohlenstoffatomen bedeutet.

3. Kraftstoffzusammensetzung nach Anspruch 1, wobei das metallchelatisierende Mittel (Ch) ausgewählt ist aus:
(A) aromatischen Mannichbasen, nämlich einem Reaktionsprodukt aus (A-1) einem mit Kohlenwasserstoff substituierten aromatischen Phenol oder Thiophenol, (A-2) einem Aldehyd oder einem Keton und (A-3) einem Amin mit mindestens einer primären- oder sekundären Aminogruppe,
(B) Aminosäureverbindungen der Formel in der R₁ ein Wasserstoffatom oder einen Kohlenwasserstoffrest bedeutet; R₂ den Rest R₁ oder einen Acylrest darstellt; R₃ und R₄ jeweils unabhängig voneinander Wasserstoffatome oder Niederalkylreste bedeuten; und z 0 oder 1 ist,
(C) β-Diketonen, gekennzeichnet durch die Formel
R-C(O)-CH₂-C(O)-R₁ (VII)
in der R und R₁ jeweils unabhängig voneinander Kohlenwasserstoffreste darstellen;
(D) Phenolverbindungen der Struktur in der jeder Rest R einen Kohlenwasserstoffrest bedeutet; und X die Gruppe CH₂, S oder CH₂OCH₂ bedeutet, und
(E) einer aromatischen difunktionellen Verbindung der Formel: in der R¹ einen Kohlenwasserstoffrest mit 1 bis 100 Kohlenstoffatomen darstellt, n eine ganze Zahl von 0 bis 4 bedeutet; Y sich bezüglich X in der ortho- oder meta-Stellung befindet; und X und Y jeweils unabhängig voneinander die Gruppen OH, NR₂, NHR, COOR, SH oder C(O)H bedeuten, in denen R ein Wasserstoffatom oder einen Kohlenwasserstoffrest bedeutet.

4. Kraftstoffzusammensetzung nach Anspruch 3, wobei die aromatische Phenol- oder Thiophenolverbindung (A-1) wiedergegeben wird durch die Formel: in der Ar einen aromatischen Rest oder einen angekuppelten aromatischen Rest bedeutet; m 1, 2 oder 3 ist, n eine ganze Zahl von 1 bis 4 bedeutet; R¹, unabhängig voneinander, ein Wasserstoffatom oder einen Kohlenwasserstoffrest mit 1 bis 100 Kohlenstoffatomen bedeutet; R° ein Wasserstoffatom oder eine Amino- oder Carboxylgruppe bedeutet und X die Gruppen O, S oder beide bedeutet, falls m 2 oder größer ist;
wobei der Aldehyd oder das Keton (A-2) gekennzeichnet ist durch die Formel: in der R² und R³ unabhängig voneinander Wasserstoffatome oder Kohlenwasserstoffreste mit 1 bis 18 Kohlenstoffatomen bedeuten oder R³ einen Carbonylgruppen-haltigen Kohlenwasserstoffrest mit 1 bis 18 Kohlenstoffatomen darstellt;
wobei die (A-3)-Verbindung ein Kohlenwasserstoffamin mit 0 bis 10 Hydroxyl- und Thiolgruppen und 1 bis 10 Aminogruppen darstellt;
wobei für die Aminosäure (VI) R¹ einen Alkyl-, Cycloalkyl-, Phenyl-, alkylsubstituierten Phenyl-, Benzyl- oder alkylsubstituierten Benzylrest bedeutet;
R₃ und R₄ Wasserstoffatome bedeuten; z null ist und
R₂ einen Acylrest der Formel:
R₂'C(O)-
bedeutet, in der R₂' einen aliphatischen Rest mit bis zu 30 Kohlenstoffatomen darstellt und wobei in der phenolischen Verbindung (VIII) der Rest X die Gruppe CH₂ darstellt, und jeder der Reste R einen Kohlenwasserstoffrest mit 4 bis 20 Kohlenstoffatomen bedeutet.

5. Kraftstoffzusammensetzung nach Anspruch 4,
wobei R¹ in der (A-1)-Verbindung ein Wasserstoffatom, einen Alkylrest mit 1 bis durchschnittlich 70 Kohlenstoffatomen, Alkenylrest mit 2 bis 30 Kohlenstoffatomen, Cycloalkylrest mit 4 bis 10 Kohlenstoffatomen, aromatischen Rest mit 6 bis 30 Kohlenstoffatomen, aromatisch substituierten Alkyl- oder alkylsubstituierten aromatischen Rest mit 7 bis 30 Kohlenstoffatomen bedeutet, und das Kupplungsmittel des angekuppelten Ar-Restes eine O, S, NH oder eine Niederalkylengruppe darstellt;
wobei das Amin (A-3) mindestens ein aliphatisches oder aromatisches Monoamin oder Polyamin mit mindestens einer primären und/oder sekundären Aminogruppe, ein Polyalkylenpolyamin oder heterocyclisches Amin oder Polyamin ist.

6. Kraftstoffzusammensetzung nach Anspruch 3, wobei (A-3) ein Hydroxykohlenwasserstoffamin mit der Formel: bedeutet, in der jeder der Reste R¹ unabhängig voneinander ein Wasserstoffatom oder einen Kohlenwasserstoff-, Hydroxykohlenwasserstoff-, Aminokohlenwasserstoff- oder Hydroxyaminokohlenwasserstoffrest bedeutet, mit der Maßgabe, daß mindestens einer der Reste R¹ einen Hydroxykohlenwasserstoff- oder Hydroxyaminokohlenwasserstoffrest darstellt; R² eine Alkylengruppe bedeutet und x eine ganze Zahl von 0 bis 5 bedeutet.

7. Titan- oder Zirkoniumkomplex, gekennzeichnet durch die Formel
(RO)ₓM(Ch)_{y} (I)
in der R ein Wasserstoffatom oder einen Kohlenwasserstoffrest mit 1 bis 30 Kohlenstoffatomen bedeutet; M ein Titan- oder Zirkoniumatom bedeutet; x 1 oder 2 ist; y 2 oder 3 ist; x + y 4 ist; und Ch abgeleitet ist von einem metallchelatisierenden Mittel ausgewählt aus:
(A) aromatischen Mannich-Basen, die Reaktionsprodukte aus (A-1) einem mit einem Kohlenwasserstoff substituierten aromatischen Phenol oder Thiophenol, (A-2) einem Aldehyd oder Keton und (A-3) einem Amin, welches mindestens eine primäre oder sekundäre Aminogruppe enthält, sind.

8. Komplex nach Anspruch 7,
wobei (A-1) wiedergegeben wird durch die Formel: in der Ar einen aromatischen Rest oder angekuppelten aromatischen Rest bedeutet; m 1, 2 oder 3 ist, n eine ganze Zahl von 1 bis 4 bedeutet; R¹, unabhängig voneinander, ein Wasserstoffatom oder einen Kohlenwasserstoffrest mit 1 bis 100 Kohlenstoffatomen bedeutet; R° ein Wasserstoffatom, eine Amino- oder Carboxylgruppe darstellt, und X die Gruppe O, S oder beide bedeutet, falls m 2 oder größer ist;
wobei (A-2) gekennzeichnet ist durch die Formel: oder eine Vorstufe davon, in der R² und R³ unabhängig voneinander Wasserstoffatome oder einen Kohlenwasserstoffrest mit 1 bis 18 Kohlenstoffatomen bedeuten, oder R³ einen Carbonylgruppen-haltigen Kohlenwasserstoffrest mit 1 bis 18 Kohlenstoffatomen bedeutet;
wobei (A-3) gekennzeichnet ist durch die Formel in der R¹ einen Kohlenwasserstoff-, aminosubstituierten Kohlenwasserstoff-, hydroxysubstituierten Kohlenwasserstoff- oder alkoxysubstituierten Kohlenwasserstoffrest bedeutet und R² ein Wasserstoffatom oder den Rest R¹ darstellt.

9. Kraftstoffadditivkonzentrat, umfassend ein normalerweise flüssiges, organisches Verdünnungsmittel und 10 bis 99 Gew.-% des Komplexes nach einem der Ansprüche 7 und 8.

10. Verfahren zum Betreiben eines Dieselmotors, der mit einem Abgassystem mit Partikelfänger ausgerüstet ist, um das Entstehen von Abgaspartikeln, die sich in dem Fänger anreichern, zu vermindern, umfassend den Betrieb des Dieselmotors mit einem Kraftstoff nach einem der Ansprüche 1 bis 6.

11. Verfahren zum Betreiben eines Dieselmotors, der mit einem Abgassystem mit Partikelfänger ausgerüstet ist, um das Entstehen von Abgaspartikeln, die sich in dem Fänger anreichern zu vermindern, umfassend den Betrieb des Dieselmotors mit einem Kraftstoff, enthaltend mindestens einen der Titan- oder Zirkoniumkomplexe nach einem der Ansprüche 7 bis 8.

## Revendications

1. Une composition de carburant comportant une quantité prépondérante d'un carburant diesel, liquide sous les conditions normales, et une quantité plus faible, destinée à l'amélioration des caractéristiques, d'au moins un complexe de titane ou de zirconium, efficace pour abaisser la température d'allumage des particules d'échappement recueillies dans les pièges à particules de systèmes d'échappement de moteur diesel, caractérisée par la formule :
(RO)ₓM(Ch)_{y} (I)
dans laquelle R est de l'hydrogène ou un groupe hydrocarbyle renfermant de 1 à 30 atomes de carbone; M est du titane ou du zirconium, x est 1 ou 2; y est 2 ou 3; x + y est 4; et, Ch est dérivé d'au moins un agent de chélation de métaux.

2. La composition de carburant selon la revendication 1, dans laquelle l'agent chélatent (Ch) est un diol, un dithiol, un mercapto-alcool, une diamine, un amino-alcool, un amino-thiol, un orthoaminophénol, un acide dicarboxylique, un acide hydroxy carboxylique, un acide mercapto carboxylique, un acide amino carboxylique, une dicétone, un acide cétocarboxylique ou un ester, ou bien des mélanges de ceux-ci;
dans laquelle le complexe est un complexe de titane; et,
dans laquelle R dans la figure 1 est un groupe aliphatique renfermant de 1 à 30 atomes de carbone.

3. La composition de carburant selon la revendication 1, dans laquelle l'agent de chélation de métaux (Ch) est choisi parmi:
(A) Les bases aromatiques de Mannich, qui sont chacune le produit de la réaction de (A-1) un phénol aromatique substitué par un hydrocarbone ou un thiophénol, de (A-2), un aldéhyde ou une cétone, et de (A-3) une amine qui contient au moins un groupe amino primaire ou secondaire;
(B) les composés amino-acides de la formule dans laquelle R₁ est de l'hydrogène ou un groupe hydrocarbyle; R₂ est R₁ ou un groupe acyle; R₃ et R₄ représentent chacun indépendamment, de l'hydrogène ou des groupes alkyle inférieur; et z est 0 ou 1,
(C) des béta-dicétones caractérisées par la formule:
R-C(O)-CH₂-C(0)-R₁ (VII)
dans laquelle R et R₁ représentent chacun indépendamment des groupes hydrocarbyles;
(D) Les composés phénoliques de la structure dans laquelle chaque R est un groupe hydrocarbyle; et x est CH₂, S, ou CH₂OCH₂, et
(E) les composés aromatiques difonctionnels de la formule : dans laquelle R¹ est un groupe hydrocarbyle renfermant de 1 à 100 atomes de carbone, n est un nombre entier de 0 à 4; Y se trouve dans une position ortho ou méta par rapport à X; et X et Y représentent chacun indépendamment des groupes OH, NR₂, NHR, COOR, SH ou C(0)H, dans lesquels R est de l'hydrogène ou un groupe hydrocarbyle.

4. La composition de carburant de la revendication 3, dans laquelle le composé aromatique phénol ou thiophénol (A-1) est représenté par la formule: dans laquelle Ar est un groupe aromatique ou un groupe aromatique couplé; m est 1, 2 ou 3, n est un nombre entier de 1 à 4; R¹, indépendamment, est de l'hydrogène ou un groupe hydrocarbyle possédant de 1 à 100 atomes de carbone; R° est de l'hydrogène, un groupe amino ou un groupe carboxyle, et x est 0, S, ou bien les deux lorsque m est 2 ou supérieur à 2;
dans laquelle l'aldéhyde ou la cétone (A-2) est caractérisée par la formule : dans laquelle R² et R³ représentent, indépendamment, de l'hydrogène, un groupe hydrocarbone présentant de 1 à 18 atomes de carbone, ou R³ est un groupe hydrocarbone renfermant du carbonyle, présentant de 1 à 18 atomes de carbone;
dans laquelle ledit composé (A-3) est une amine hydrocarbylée renferment de 0 à 10 groupes hydroxyle et thiol et de 1 à 10 groupes amine;
dans laquelle, pour l'amino acide (VI), R¹ est un groupe alkyle, cycloalkyle, phényle, phényle substitué par un alkyle, benzyle ou bien un groupe benzyle substitué par de l'alkyle;
R₃ et R₄ représentent de l'hydrogène; z est O; et
R₂ est un groupe acyle représenté par la formule
R₂ʼC(O) -
dans laquelle R₂' est un groupe aliphatique renfermant jusqu'à 30 atomes de carbone; et dans laquelle, pour le composé phénolique (VIII), X est CH₂,
et chaque R est un groupe hydrocarbyle renfermant de 4 à 20 atomes de carbone;

5. La composition de la revendication 3,
dans laquelle R¹ dans ledit composé (A-1) est de l'hydrogène, un groupe alkyle présentant de 1 jusqu'à une moyenne de 70 atomes de carbone, un groupe alcényle présentant de 2 à 30 atomes de carbone, un groupe cycloalkyle présentant de 4 à 10 atomes de carbone, un groupe aromatique présentant de 6 à 30 atomes de carbone, un groupe alkyle substitué par un radical aromatique ou un groupe aromatique substitué par un radical alkyle présentant de 7 à 30 atomes de carbone, et ledit agent de couplage dudit groupe couplé Ar est 0, S, NH ou un groupe alcylène inférieur;
dans laquelle l'amine (A-3) est au moins une monoamine ou une polyamine aliphatique ou aromatique renfermant au moins un groupe amine primaire et/ou secondaire, une polyalcylène polyamine, ou bien une amine ou une polyamine hétérocyclique.

6. La composition de carburant de la revendication 3, dans laquelle (A-3) est une hydroxylhydrocarbyl amine présentant la formule : dans laquelle chacun des R¹ représente indépendamment un atome d'hydrogène ou un groupe hydrocarbyle, hydroxyhydrocarbyle, aminohydrocarbyle ou hydroxyaminohydrocarbyle, sous la condition qu'au moins l'un des R¹ soit un groupe hydroxyhydrocarbyle ou hydroxyaminohydrocarbyle; R² est un groupe alkylène et x est un nombre entier de 0 à 5.

7. Un complexe de titane ou de zirconium caractérisé par la formule:
(RO)ₓM(Ch)_{y} (I)
dans laquelle R est de l'hydrogène ou un groupe hydrocarbyle renfermant de 1 à 30 atomes de carbone; M est du titane ou du zirconium; x est 1 ou 2; y est 2 ou 3; x + y est 4; et Ch est dérivé d'un agent d chélation de métaux choisi parmi :
(A) des bases aromatiques de Mannich, qui sont les produits de la réaction (A-1) un phénol ou thiophénol aromatique substitué par un radical hydrocarbone, (A-2) un aldéhyde ou une cétone, et (A-3) une amine qui renferme au moins un groupe amino primaire ou secondaire.

8. Le complexe de la revendication 7,
dans lequel (A-1) est représenté par la formule : dans laquelle Ar est un groupe aromatique ou un groupe aromatique couplé; m est 1, 2 ou 3, n est un nombre entier de 1 à 4; R¹, indépendamment, représente de l'hydrogène ou un groupe hydrocarbyle possédant de 1 à 100 atomes de carbone; R° est de l'hydrogène, un radical amino ou un radical carboxyle et X est 0,S, ou bien les deux lorsque m est 2 ou supérieur à 2;
dans laquelle (A-2) est caractérisé par la formule: ou bien un précurseur de celui-ci dans laquelle R² et R³, indépendamment, représentent de l'hydrogène, un groupe hydrocarbyle possédant de 1 à 18 atomes de carbone, ou R³ est un groupe hydrocarbone renfermant du carbonyle, présentant de 1 à 18 atomes de carbone;
dans laquelle (A-3) est caractérisé par la formule dans laquelle R¹ est un groupe hydrocarbyle, hydrocarbyle substitué par un radical amino, hydrocarbyle substitué par un radical hydroxy, ou bien un groupe hydrocarbyle substitué par un radical alkoxy, et R² est de l'hydrogène ou R¹.

9. Un concentré d'additif pour carburant comportant un diluant organique liquide sous les conditions normales et de 10 à 99% en poids du composé tel que revendiqué dans l'une des revendications 7 et 8.

10. Une méthode pour faire fonctionner un moteur diesel équipé d'un système de piège pour particules d'échappement afin de réduire l'accumulation des particules d'échappement collectées dans ledit piège, méthode dans laquelle on fait fonctionner ledit moteur diesel avec un carburant tel que revendiqué dans l'une quelconque des revendications 1 à 6.

11. Une méthode pour faire fonctionner un moteur diesel équipé d'un système de piège pour particules d'échappement afin de réduire l'accumulation des particules d'échappement collectées dans ledit piège, méthode dans laquelle on fait fonctionner ledit moteur diesel avec un carburant renfermant au moins un des complexes de titane ou de zirconium selon l'une quelconque des revendications 7 à 8.
